

Apr. 3, 1923.

1,450,725

F. HODSON

ELECTRICAL RESISTANCE HEATING ELEMENT AND PROCESS OF MAKING SAME

Filed May 22, 1922

*Fig. 1.*



*Fig. 2.*



*Fig. 3.*



Witnesses

Geo. A. Gross  
Augustus B. Cope

Inventor  
Frank Hodson

By Joshua R. T. Tott  
his Attorney

## UNITED STATES PATENT OFFICE.

FRANK HODSON, OF PHILADELPHIA, PENNSYLVANIA.

## ELECTRICAL RESISTANCE HEATING ELEMENT AND PROCESS OF MAKING SAME.

Application filed May 22, 1922. Serial No. 562,568.

To all whom it may concern:

Be it known that I, FRANK HODSON, a subject of the King of Great Britain, residing at Philadelphia, in the county of Philadelphia and State of Pennsylvania, have invented certain new and useful Improvements in Electrical Resistance Heating Elements and Process of Making Same, of which the following is a specification.

- 10 My present invention relates to electrical resistance heating elements and particularly to the kind made of amorphous or graphitic carbon capable of being used as heating agents in electric furnaces of various types.
- 15 One object of the present invention is to provide improved means for obviating the oxidizing of resistance elements. Another object is to make the mechanical strength of such elements so as to enable the use 20 thereof in a practical capacity within furnaces or the like.

Generally speaking the preferred process of making my improved elements consists in placing an electrical resistance heating element, such for example as a helical coil of graphite, in a suitable mold of any shape or design and ramming powdered or granular silicon-carbide, which has been previously mixed with a small proportion of suitable clay or other binding material, between the element and the mold to give the desired thickness of silicon-carbide over the whole of the element. The mold may be made of any suitable material such for example as carborundum. The element is then heated either from an external source or preferably by passing a current of electricity through the element until the element and its covering are heated to a temperature necessary to 35 form the whole into a solid mass; the element then being encased in a highly refractory and practically non-oxidizing envelope.

The envelope may be made absolutely impervious by glazing the surface with high temperature glaze. This may be carried out by coating the mold with the glaze before ramming the silicon-carbide mixture.

Specifically speaking I attain the above mentioned objects in the following manner, reference being had to the accompanying drawing in which—

Figure 1 is a side view of an electric resistance heating element made in accordance with my invention; the same being made out 55 of graphite or other form of carbon including a helical coil,

Figure 2 is a view partly in longitudinal central section illustrating the element of Figure 1 enclosed in its highly refractory envelope, and

Figure 3 is a transverse section taken on the line 3—3 of Figure 2.

Referring to the drawing, the element 4 can be made by turning the same from a bar of graphite or other form of carbon to include a helically coiled portion 5 and screw threaded end portions 6 and 7. The helically coiled portion 5 is placed within a mold such for example as a cylindrical mold 8 of carborundum as shown in Figures 2 and 3; said mold being of larger internal diameter than the external diameter of the helically coiled portion 5 of the element 4. The space between the convolutions of said coiled portion and the space between said coiled portion and the inner surface of the mold 8 is then rammed with said silicon-carbide mixture illustrated at 9. If desired, rings 10 and 11 can be screwed on the end portions 6 and 7 to form an end abutment for the mold 8 and silicon-carbide mixture. The structure thus formed is heated as above stated to a temperature necessary to form the whole into a solid mass and the element 4 is then encased in a highly refractory and practically non-oxidizing envelope. The structure thus produced can be used as an electrical resistance heating means in which the electric current can be utilized so as to pass through the element 4 taking the path of 90 the helical convolutions of the coil 5; thus creating heat. At the same time oxidizing of the element is practically impossible and sufficient strength is imparted thereto to prevent the breaking down of the element 95 during use.

While I have described my invention as taking a particular form, it will be understood that the various parts of my invention may be changed without departing from the spirit thereof, and hence I do not limit myself to the precise construction set forth, but consider that I am at liberty to make such changes and alterations as fairly come within the scope of the appended claims.

Having thus described my invention, what I claim as new and desire to secure by Letters Patent is:—

1. An electrical resistance heating element including a coil of carbon.
2. An electrical resistance heating element including a coil of graphite.

3. An electrical resistance heating element including a helical coil of carbon.
  4. An electrical resistance heating element including a helical coil of graphite.
  5. An electrical resistance heating element including a coiled portion of carbon enclosed in an envelope of highly refractory material.
  6. An electrical resistance heating element including a coiled portion of graphite enclosed in an envelope of highly refractory material.
  7. An electrical resistance heating element including a helically coiled portion of carbon enclosed in an envelope of highly refractory material.
  8. An electrical resistance heating element including a helically coiled portion of graphite enclosed in an envelope of highly refractory material.
  9. The process herein described consisting of taking an electrical resistance element encasing said element in a non-oxidizing and highly refractory covering and then heating the same.
- 25
10. The process herein described consisting of taking an electrical resistance element encasing said element in a non-oxidizing and highly refractory covering including silicon-carbide and then heating the same.
  11. The process herein described consisting of the placing of an electrical resistance heating element in a mold, then filling the space between said element and said mold with highly refractory material and then heating the structure thus formed.
- 30
- 35
- In testimony whereof I have signed my name to this specification in the presence of two subscribing witnesses.
- 40

FRANK HODSON.

Witnesses:

A. EVERHARDT,  
HORACE DREVER.